

UNITED STATES PATENT OFFICE

PAUL VIRCK, OF DESSAU IN ANHALT, GERMANY, ASSIGNOR TO GENERAL ANILINE  
WORKS, INC., OF NEW YORK, N. Y., A CORPORATION OF DELAWARE

## PROCESS OF DYEING PELTS, HAIRS, FEATHERS, AND THE LIKE

Application filed December 6, 1927, Serial No. 238,221, and in Germany September 14, 1926.

I have filed applications for this patent in Germany Sept. 14, 1926; Austria, Nov. 4, 1927; Poland, Nov. 9, 1927. with an aqueous solution of a salt of a naphthalene derivative of the general formula: 
$$\text{X}_1 \text{X}_2$$

1921, Poland, Nov. 9, 1921.  
This invention relates to a process of dyeing pelts, hairs, feathers and the like with a naphthalene derivative which contains as a substituent a 3-amino-aryl-amino-group of the benzene series. The naphthalene residue may also contain a substituent or substituents such as a hydroxy-group, an amino-group or an amino-aryl-amino-group.

The compounds used according to my invention for the purpose set forth correspond to the general formula:

15



20 wherein X means H, alkyl or halogen and Y stands for H,  $-\text{OH}$ ,  $-\text{NH}_2$ , or  $-\text{NH-aryl-NH}_2$ .

The not mordanted goods are treated with  
25 an aqueous solution of a salt of such a 3-amino-aryl-amino-derivative of the naphthalene and then with an acid nitrite solution, whereby valuable dyeings are produced on the fiber. For example, a thoroughly killed  
30 skin is handled at ordinary temperature for some hours in a bath containing per liter 2 gr. of 2-(3'-aminophenylamino)-naphthalene hydrochloride, some alcohol and a small proportion of hydrochloric acid. It is then washed  
35 and handled in a second bath containing per liter 3 grams of sodium nitrite and 6 grams of acetic acid per liter. The dyeing is between yellow and rose.

40 2-(4'-methyl-3'-aminophenylamino)-naphthalene produces a similar dyeing, 2-(4'-methyl-3'-aminophenylamino)-7-hydroxynaphthalene produces a reddish-brown dyeing.

45 Similar dyeings are obtained from the naphthalene derivatives mentioned which are substituted in the benzol nucleus by halogen.

What I claim is:—

1. A process of dyeing pelts, hairs and feathers by successively treating the goods



(wherein X means H or an univalent substituent of the group consisting of alkyl and halogen and wherein Y means H or an univalent substituent of the group consisting of  $-\text{OH}$ ,  $-\text{NH}_2$ ,  $-\text{NH}-\text{aryl}-\text{NH}_2$ ) and with an acid nitrite solution.

2. A process of dyeing pelts, hairs and feathers by successively treating the goods with an aqueous solution of a salt of a naphthalene derivative of the general formula: 65



(wherein X means H or an univalent substituent of the group consisting of alkyl and halogen), and with an acid nitrite solution.

3. A process of dyeing pelts, hairs and feathers by successively treating the goods with an aqueous solution of 2-(3'-aminophenylamino) naphthalene hydrochloride and with an acid nitrite solution. 75

In testimony whereof, I affix my signature. 80  
PAUL VIRCK.

85

90

95

100